

Nov. 6, 1928.

1,690,474

L. W. CAFFERATA

METHOD OF MAKING REINFORCED BLOCKS

Filed June 15, 1925

*Fig.1*



2

1

*Fig. 2*



2

M'

*Fig. 3*



*Inventor*  
*Louis W. Cafferata*

*George S. Scarff.*

*By*

*Attorney*

## UNITED STATES PATENT OFFICE.

LOUIS WILLIAM CAFFERATA, OF NEWARK-ON-TRENT, ENGLAND.

## METHOD OF MAKING REENFORCED BLOCKS.

Application filed June 15, 1925. Serial No. 37,177.

The general subject matter of my present invention is the production of a new type of plaster block or building block especially such as having plaster or lime or a combination of each as its principal cementing medium. With such I combine as a novel reenforcement, a fibrous medium of non-rigid form, in such a way as greatly to increase the strength of the block while preserving and 10 even increasing certain other characteristics.

The several elements of novelty, in my invention, appear in the product, in certain desirable characteristics of product incident to its use and generally in a system of reenforcement with the resilient, fibrous material introduced into the plastic composition of the block and fabricated therein during the process of pouring and molding of the block or slab.

20 The so-called gypsum block or plaster block or tile has been familiarly known and increasingly used in the building material and construction trades in recent years. From a small beginning the growth in the use 25 of this product has been rapid, until at the present time many million square feet of these block or tile are being used each year in the United States, for construction work as partition tile and general insulating pur- 30 poses.

These gypsum blocks or tiles are manufactured from commercial plaster of Paris by mixing approximately equal proportions of the plaster of Paris and water and 35 pouring the mixed magma into molds, having removable rods or mandrels which serve the purpose of making the core holes in the block. Practically all of the plaster blocks manufactured in the United States, above 40 the two inch thickness, are made in hollow form or having core holes or hollows. The purpose of the hollows is to make a lighter block and at the same time to use a lesser amount of plaster of Paris per given unit 45 of block. Also, a hollow block dries or cures more quickly than the solid block. The breakage, however, in removing these hollow blocks from their molds and in further handling them during process of transportation to the job, is very considerable.

50 My invention contemplates the elimination

of or reduction in breakage and at the same time greatly increasing the compressive strength and toughness of plaster blocks, by the reenforcing of the block throughout its 55 length and breadth by embedding in the plaster mixture, during process of pouring, a fibrous, non-rigid substance such as rush reeds, or rattan fibre or similar materials of cellulose composition.

60 To such a fibrous material the plaster composition bonds tenaciously, even during the preliminary casting and hardening of the plaster composition used in the blocks, to such an extent that within fifteen to twenty 65 minutes after pouring the plaster magma in molds or on continuous belts, and thereby forming a reenforced plaster block or slab, said slab may be sawed or otherwise cut into standard lengths without breaking the bond 70 between the fibre reenforcement and the plaster mixture.

75 Another advantage of this fibre reenforcement is due to its resiliency which permits the plaster block or slab thus reenforced to show a certain deflection or bending movement without breaking away from the plaster bond.

80 Fibrous material such as the rush reed, or rattan fibre strands are porous in texture and when embedded within a plaster mixture, suitable for blocks, permit an immediate inter-growth of the plaster crystal among the interstices of the fibre reenforcement and to this fact, as well as to the rough texture of 85 these reeds or rattan strands, great binding strength is derived.

90 Another feature of my fibre reenforced blocks is in their lightness as compared to a solid non-reenforced block or slab, as the fibre strands distributed throughout the width of the block or slab replace just so much of the heavier plaster mixture, lightening the block and to all intents and purposes serve the same as the core holes in the hollow 95 block but give more than double the strength of the hollow block.

100 I find again that for certain types of plaster, such as the plaster recovered from by-product or precipitated gypsum, which when converted into plaster of Paris, is inclined to be very finely divided and makes a more

porous and less dense plaster slab. Said slab made from such plaster is apt to be weak and the only possible way of manufacturing a plaster block which will pass standard specifications for strength, from such plaster, is by my fibre reenforcement. Furthermore, such reenforcement is practically self-adjusting for position in the block so as to require very little manipulation and in spite of its strength is severable without difficulty and without disturbance of its relation in the block.

To make my invention clear in its general applicability, I will show and discuss the 15 plaster block instance above referred to, as that is not only indicative of general use, but in itself is a highly successful specific case. Throughout the specification and drawings like reference characters are employed 20 to indicate corresponding parts, and in the drawings:

Fig. 1 is a sectional view of a block in accordance with my invention.

Fig. 2 a diagrammatic view showing the 25 characteristic formation of a block slab, and Fig. 3 a similar view showing the cutting of the same.

For a block or unit illustrative of my invention I have shown a block of general type, 30 rectangular in cross section and of greater length than height or breadth. I show such a form as it is characteristic. Within this block 1 I have indicated at 2 my reenforcement which is shown as extending generally 35 longitudinally of the block and in general parallelism, although I have shown this as being somewhat irregular as there is an advantage in having the individual reenforcing units disposed in somewhat of a crossed relation so as to secure a greater bonding 40 and a greater resistance to strains which are apt to be symmetrical to the faces of the block.

This reenforcement 2 is introduced during 45 the molding as indicated in Fig. 2 of the drawings. In these drawings I have shown a belt type of mold consisting of lateral mold pieces M and a bottom M<sup>1</sup> into which the mixed plaster of Paris or like material is discharged in fluid state from a container C. The discharge is so timed and regulated as 50 to fill the belt mold as it moves along the course of its travel, which is of sufficient length to give the plaster time to set before it is cut up.

This brings us to the point of the type of 55 reenforcement contemplated by my invention. For that purpose, I utilize sections of plant growth in the form of stalks or sheets. There are a great variety of such growths more or less available and of more or less desirability as regards several factors that are controlling. It is impossible for me to catalog here all of such growths, but I will 60 first describe the desired characteristic and

then give instances of some of those that seem most satisfactory.

In the first place, such growth is preferably light and of considerable buoyancy and either by its nature free from bark or husk 70 or readily stripped thereof. It is preferably of strong longitudinal fibre and while absolute straightness is not necessary, a general straightness is desirable and convenient. For the best results the surface should be easily 75 wetted and preferably permeable by water so as to increase the efficiency of the bonding of the reenforcement in the wet plaster as it is being molded.

The best materials for this purpose are 80 those shoots of the palm family that grow rapidly, such as some of the bamboos or, according to my experience as most desirable, the so-called rattan. Rattan not only combines the desired characteristics above 85 enumerated, but is available in the waste from rattan manufactures where the shorter pieces are not usable and have heretofore been regarded in large part as waste.

Considering now such a material, it will be 90 seen that it can be laid in the molds as they are filled with the fluid plaster, extending longitudinally and largely in a natural arrangement by their individual power of flotation. I have indicated at P any means of 95 submerging this reenforcement and this submerging action usually should continue until the plaster begins to set slightly so as to secure a distribution of the reenforcement through the block in the direction of its 100 depth.

The reenforcement should be laid in preferably with a slight overlapping or splicing effect so that the reenforcement longitudinally of the slab for any given length will be 105 practically continuous in its overlapped, as well as its interlaced condition. This produces in the slab a reenforcement of great continuity and strength.

The cutting of such a slab so reenforced 110 may be accomplished without the slightest difficulty or the slightest disturbance to the bonding of the reenforcement. I have indicated at S a saw which is moved intermittently to cut the slab into sections of the desired length. These may then be loaded on trucks and run through driers where the final setting is completed. Such blocks are of great strength and lightness and are producible at low cost.

Various modifications may obviously be made in the form of the block and in the manner of its formation, as well as in the selection of the material to be used as reenforcement, all without departing from the 115 spirit of my invention if within the limits of the appended claims.

What I therefore claim and desire to secure by Letters Patent is:

1. The method of making plaster of Paris 130

blocks, consisting in placing in a mold a buoyant reenforcement and in filling the mold with fluid plaster and keeping the re-enforcement submerged until held by the set 5 of the plaster.

2. The method of making plaster of Paris blocks consisting in feeding to a moving mold a reenforcement of plant stalks disposed lon-

gitudinally thereof, in filling the mold with fluid plaster as it moves to form a slab with 10 the reenforcement embedded therein, and in transversely cutting the slab into blocks of the required length.

In testimony whereof I affix my signature.

LOUIS WILLIAM CAFFERATA.